

Patented Nov

2,302,616

November 11, 1942

# UNITED STATES PATENT OFFICE

2,302,616

## BRIQUETTE FOR THE ADDITION OF TUNGSTEN TO FERROUS ALLOYS

Arthur Linz, New York, N. Y., assignor to Climax Molybdenum Company, New York, N. Y., a corporation of Delaware

No Drawing. Application April 22, 1941,  
Serial No. 389,752

6 Claims. (Cl. 75—133)

The present invention relates to a novel and improved addition agent for the production of tungsten containing ferrous alloys.

Objects and advantages of the invention will be set forth in part hereinafter and in part will be obvious herefrom, or may be learned by practice with the invention, the same being realized and attained by means of the compositions, steps, processes and instrumentalities pointed out in the appended claims.

The invention consists in the novel compositions, steps, processes combinations and improvements herein shown and described.

The present invention has for its objects the provision of a novel and improved tungsten containing alloying agent which is generally useful for the production of tungsten containing ferrous alloys. The invention further provides a novel and improved tungsten briquette which can be economically produced and contains a minimum of foreign material. The invention has for another object the provision of an improved tungsten containing briquette which can be used practically all places where other tungsten addition agents have heretofore been used, and which is superior in one respect or another to all of the previous tungsten addition agents.

Heretofore tungsten has been added to ferrous alloys, by a large number of different processes involving a wide variety of different addition agents. Tungsten ores and concentrates as well as calcium tungstate have been proposed and used as an addition agent but have proved to be of very limited application due to the relatively large proportion of slag and other undesirable constituents contained therein and introduced thereby into the ferrous alloy. Tungsten trioxide, dioxide and other oxides have all been used as addition agents, but their use has almost invariably been attended by excessive loss of tungsten, resulting in increased cost of producing the alloy, and furthermore their use has been limited to the production of ferrous alloys to contain a small amount of tungsten.

Ferro-tungsten has also been widely used for the production of tungsten-bearing ferrous alloys, and while there is no limit to the amount of tungsten which may be contained in the alloys produced therewith, this type of addition agent has necessarily increased the cost due to the added operations required for the manufacture of ferro-tungsten. Furthermore, ferro-tungsten has the disadvantage that it sinks to the bottom of the ladle and the resulting ferrous alloy is rendered homogeneous only with difficulty.

Briquettes of tungstic oxides with carbon have been widely used, and while they avoid many of the disadvantages of the other alloying agents, they produce a boil, and when large percentages of tungsten are to be added in this way, the gas evolution may be excessive. Tungsten silicides have also been used as addition agents where a fairly high silicon content in the resulting alloy is unobjectionable.

10 In general, the various ways in which tungsten has been added to ferrous alloys have been substitutes for the universally usable ferro-tungsten, which has its relatively high cost and its relatively high specific gravity, as its principal commercial disadvantages.

15 In addition to the foregoing, there have been other minor ways proposed for the addition of tungsten to ferrous alloys, but these have not met with any considerable commercial use.

20 The present invention provides an economical tungsten addition agent for ferrous alloys, which eliminates the use of any relatively expensive reducing agents, the availability of which may be restricted, such as aluminum, silicon, magnesium and calcium, requires a minimum of equipment for its production, eliminates the objections which have existed with respect to all of the commercially used addition agents set forth above, and does not result in the introduction into the molten ferrous metal of any foreign material.

25 Thus, the tungsten addition agent of the present invention provides a universally acceptable tungsten containing compound for the introduction of tungsten into ferrous alloys which can be used, with considerable savings, as a substitute for any of the tungsten addition agents heretofore found useful, thereby simplifying the production of tungsten addition agents in general, as well as reducing the variety of such addition agents which must be carried on hand by the manufacturer or steel maker.

30 In accordance with the present invention, crude tungstic oxide is partially reduced to form crude lower tungsten oxides, or crude tungsten metal powder containing some of the lower tungsten oxides as impurities, and this oxide is mixed intimately with relatively fine powdered, granular or flake-like iron. The resultant intimate mechanical mixture of these substances is highly compressed to form briquettes which are preferably of uniform size. Due to the peculiar and dissimilar characteristics of the tungsten compound and the iron particles, no foreign binder is needed for the coherence of this mixture, and

the briquettes preferably contain not more than a trace of carbon or other impurities.

It will be understood that the foregoing general description and the following detailed description as well, are exemplary and explanatory but are not restrictive of the invention.

Referring now in detail to the present preferred and illustrative embodiments of the invention, the novel and improved tungsten containing briquettes are formed from partially reduced crude tungstic oxide. The tungstic oxide is reduced in a beehive or coke oven, and the reduction is carried on until the oxide contains mostly tungsten dioxide with some tungsten oxide, and the remainder is metallic tungsten and gangue; or, the reduction may be carried on still further until the tungsten is primarily present as metallic tungsten, with some of the other lower tungsten oxides and gangue. As used herein, the term "reduced tungstic oxide" refers to such a mixture comprising principally tungsten dioxide, tungsten oxide and metallic tungsten, while the terms "crude tungsten powder" and "highly reduced tungstic trioxide" refer to a similar mixture in which the metallic tungsten predominates. The reducing agent may conveniently be carbon or some other reducing agent such as pitch which is substantially entirely removed from the tungsten compound by the end of the reduction process. Preferably, not more than 0.25% carbon is contained in the briquettes as they are finally made up.

The reduced roasted concentrates are generally in the form of relatively small particles, the individual particles or grains having a center which is largely tungsten dioxide surrounded by a considerable layer of tungsten monoxide, which in turn is coated with the powdered metallic tungsten, these successive layers gradually merging into each other and being formed as the result of a more intensive reducing action on the surface of the particle.

The iron to be intimately mixed with the partially reduced tungsten oxides may consist of powdered granular or flakelike iron containing the normal impurities, and substantial amounts of iron oxide will not interfere with the results to be obtained.

Preferably the partially reduced tungsten oxides are mixed with from 7 to 40 per cent of the iron particles, although as little as 5 per cent or as much as 70 per cent of the iron particles may be added to the reduced tungsten oxides. This mixture is thoroughly mixed until the tungsten containing particles and the iron particles are intimately mixed, and the resulting mixture is briquetted to form relatively large briquettes which may conveniently contain a predetermined weight of tungsten. During the briquetting operation, the intimately mixed particles of the reduced tungsten oxides and the iron particles, are subjected to a relatively high pressure, and due to the different nature of the materials, the mixture is compressed into a relatively hard coherent mass which can be shipped and will stand considerable handling without excessive crumbling.

In use, the briquettes may be treated in practically the same manner as is customary with ferro-tungsten. They may be added to the steel furnace or ladle, and the tungsten is rapidly ab-

sorbed by the melting or molten steel. The briquettes sink through the slag and very slowly through the molten metal, the slag protecting the metallic tungsten from oxidation, at the same time that it allows it to be rapidly dissolved in the molten steel. Inasmuch as the briquettes do not sink rapidly to the bottom of the ladle, the resulting alloy readily and quickly becomes homogeneous, and no difficulty is experienced through slow dispersion of the tungsten throughout the alloy.

Inasmuch as the briquettes contain no foreign material, no added impurities are introduced into the alloy, and due to the fact that the tungsten is present in the briquettes in partly reduced form, the tungsten is put into the steel or iron with almost an absolute minimum of chemical reaction, only ferro-tungsten having a lesser chemical reaction. Thus, the briquettes of the present invention can replace to advantage all of the tungsten addition agents which have heretofore been used, with the added advantage that the briquettes of the present invention can be produced much more readily, and with less expense than any of the other tungsten addition agents including ferro-tungsten.

The invention in its broader aspects is not limited to the specific compositions, processes and steps described and departures may be made therefrom within the scope of the accompanying claims without departing from the principles of the invention and without sacrificing its chief advantages.

What I claim is:

1. A briquette for the addition of tungsten to ferrous alloys consisting substantially entirely of tungstic dioxide tungstic monoxide and metallic tungsten and iron particles intimately mixed together and highly compressed to form a coherent mass.
2. A briquette for the addition of tungsten to ferrous alloys consisting essentially of tungstic dioxide, tungstic monoxide and metallic tungsten in which the metallic tungsten predominates and iron particles intimately mixed together and highly compressed to form a coherent mass.
3. A briquette for the addition of tungsten to ferrous alloys consisting essentially of tungstic dioxide, tungstic monoxide and metallic tungsten in which the metallic tungsten predominates and iron particles intimately mixed together.
4. A briquette for the addition of tungsten to ferrous alloys consisting substantially entirely of tungstic dioxide tungstic monoxide and metallic tungsten and iron particles intimately mixed together and highly compressed to form a coherent mass and containing less than 0.25% carbon.
5. A briquette for the addition of tungsten to ferrous alloys consisting substantially entirely of tungstic dioxide, tungstic monoxide and metallic tungsten and 5% to 70% iron particles intimately mixed together and highly compressed to form a coherent mass.
6. A briquette for the addition of tungsten to ferrous alloys consisting substantially entirely of tungstic dioxide, tungstic monoxide and metallic tungsten and 10% to 50% iron particles intimately mixed together and highly compressed to form a coherent mass.

ARTHUR LINZ.